

## UNITED STATES PATENT OFFICE.

ALBERT H. ACKERMAN, OF CHICAGO, ILLINOIS, ASSIGNOR TO WILLIAM H. COLVIN,  
OF CHICAGO, ILLINOIS.

## PROCESS AND MATERIAL FOR TREATING METAL.

No Drawing.

Application filed March 20, 1924. Serial No. 700,710.

*To all whom it may concern:*

Be it known that I, ALBERT H. ACKERMAN, a citizen of the United States, residing in Chicago, in the county of Cook and State of Illinois, have invented a new and useful Improvement in Processes and Material for Treating Metal, of which the following is a specification.

My invention relates in general to the treatment of metals and has more particular reference to the carburizing of metals, as, for example, is required in the case-hardening of steel.

In the case-hardening of steel, the steel, after being formed, is treated in a closed chamber to cause absorption of carbon. This absorption is produced by placing within the sealed chamber, along with the steel to be treated, a charge of charcoal and coke mixed with an energizer adapted to produce the carbon-monoxide gas, from which the carbon is absorbed into the iron. These energizers in the past have consisted largely of dried, ground animal matter, as bones, hide, and the like, and none of them has proved entirely satisfactory.

The carburizing action with these compounds has required a degree of heat closely approaching the critical temperature of the metal so that the operation has been one of considerable delicacy and on this account of frequently disappointing results. Where the critical temperature is too closely approached or passed grain growth is produced in the steel which renders the product unfit for use. Other objections to the compounds usually employed prior to my invention for the carburizing of steel result from the circumstance, first, that the compounds are of uneven properties injecting an element of guesswork into the action as to the time of heat, degree of temperature, etc.; and, second, the circumstance that the energizing capacity of the compounds is relatively low and it has soon become exhausted in use.

A principal object of my present invention is the provision of an energizing material which will permit of the carburizing action either for the purpose of case-hardening or for other purposes, at a substantially lower temperature than has heretofore been practical.

Another important object of the invention is the provision of an energizer, for the purposes described, of increased active power and which may be employed a relatively greater number of times before exhaustion.

Another important object of the invention is the provision of an energizer which will produce in the steel or other metal a homogeneous carbon content prior to quenching; that will produce a uniform rate of penetration of the carbon and which, after quenching, will produce a uniform carbon content throughout the thickness of the case and a gradual and desirable diminution of the carbon content in toward the

center.

My invention contemplates both a new material and a new process of carburizing or case-hardening steel and other metals. I use as a base for my carburizing mixture natural phosphate rock giving an analysis substantially that of fossilized bone. This material, after being mined, is or may be subjected to a treatment as follows:

Dried at or about 240° to 250° F., crushed to a granular form, and then dried again at or under 300° F. The purpose of the initial drying in the process outlined above is merely to facilitate the crushing action. It may, however, be carried to a degree that will eliminate all of the moisture content, thus making unnecessary the second drying above mentioned.

Experiment has demonstrated the circumstance that this phosphate rock accomplishes all of the purposes of the invention set forth herein and has other and further advantages,—as, for example, a smaller amount may be employed to produce a given carburizing result and less ash residue results from complete exhaustion of the material. Experiment has also demonstrated that the arrangement of this material in the presence of carbon and the subjection of heat gives off the desired energizing gases at lower temperatures than has heretofore been possible—temperatures at 1200° to 1400° F. accomplishing carburization and case-hardening heretofore only accomplished within practical limits of time by temperatures of from 1650° to 1800° F.

An excellent and efficient mixture for the

carburizing or case-hardening of steel has been found to be

|                           | Per cent. |
|---------------------------|-----------|
| Coke                      | 25        |
| Charcoal                  | 35        |
| Fossilized bone energizer | 40        |
|                           | <hr/> 100 |

Such a mixture will liberate the necessary gases at a temperature well below the critical temperature of the steel being treated, will carburize the material at a uniform rate, will give a uniform carbon content prior to quenching, and will permit of use over and over again in the treatment of succeeding pieces of subject metal.

While the invention has hereinbefore been described in connection with the carburizing of steel in case-hardening, it will be obvious that both the process and the material herein described and claimed is capable of carburizing iron, steel and other metals for other purposes without departing from the spirit and scope of the invention or sacrificing all of its material advantages.

I claim:

1. A case-hardening composition, comprising, a mixture of rock phosphate, and a carboniferous substance. 30

2. A case-hardening composition, comprising, a mixture of desiccated, fossilized animal matter, and a carboniferous substance.

3. The process of case-hardening or carburizing metal, which comprises, arranging the metal to be carburized, and a carboniferous substance in a confined space and in the presence of rock phosphate, and heating. 35

4. The process of case-hardening or carburizing metal, which comprises, arranging the metal to be carburized, and a carboniferous substance in a confined space and in the presence of rock phosphate, and heating to a temperature not to exceed 1400° F. 45

5. The process of case-hardening or carburizing metal, which comprises, arranging the metal to be carburized, and a mixture of a carboniferous substance and rock phosphate in a confined space, and heating. 50

ALBERT H. ACKERMAN.